

# UNITED STATES PATENT OFFICE.

JOHN W. BODMAN, OF WESTERN SPRINGS, ILLINOIS.

## SOAP AND PROCESS OF MAKING THE SAME.

1,285,004.

Specification of Letters Patent. Patented Nov. 19, 1918.

No Drawing.

Application filed January 17, 1916. Serial No. 72,461.

*To all whom it may concern:*

Be it known that I, JOHN W. BODMAN, a citizen of the United States, residing at Western Springs, Illinois, (whose post-office address is Box 236, in Western Springs, county of Cook, and State of Illinois,) have invented new and useful Improvements in Soaps and Processes of Making the Same, of which the following is a specification.

10 This invention relates to improvements in soap and the process of making the same and more particularly to a soap containing a large part of naphtha, gasolene or other grease solvent. It has been found that ordinary soaps are not efficacious in removing the greases and oils which form a large part of most dirt. It also is a well known fact that naphtha and other petroleum derivatives, chlorin derivatives, carbon tetrachlorid, and similar substances are solvents 20 of oils and greases and when used with soap aid greatly in effecting the removal of grease and oil. I am aware of the fact that heretofore naphtha and soap have been used together in cleaning compounds and also that there have been manufactured soaps, such as naphtha soap, which contain naphtha or other grease solvent. All of such compounds and soaps, however, here- 25 tofore existing consist merely of a mixture of soap with naphtha or other grease solvent. It has been found that the proportion of grease solvent in such mixtures cannot be more than about 20% without caus- 30 ing the resulting product to lose its soapy appearance and properties. A larger proportion will fail to mix with the soap to form a homogeneous mass. It is well known also that upon exposure to the air of such products the loss of the grease solvent by evaporation is very rapid. The presence of grease solvents in the compounds heretofore known always has greatly reduced their lathering properties.

40

45 By my improved process of manufacture I am able to make a new and useful product which is soapy in appearance and action, has excellent cleaning and detergent properties and contains a large proportion (as high as 90% or 95%) of naphtha or other grease solvent and therefore is especially efficacious in removing grease and oil. Since my improved soap is not merely a mixture of ordinary soap and naphtha, or other 50 grease solvent, like the products heretofore known, but might be more accurately de-

scribed as soap in colloidal or true solution in naphtha, exposure to the air but slightly affects its appearance or condition and does not materially evaporate the naphtha. This 60 is due to the fact that the close union between the soap and naphtha causes the former to act as a binder; and to the fact that the first evaporation which occurs causes the formation of a protective coating 65 of relatively harder soap base which prevents the air from coming into contact with the rest of the body. Neither of these preventives of evaporation is found in any of the products heretofore known. They being merely mixtures with no close union between the constituent parts, the soap does not act as a binder and evaporation of the grease solvent leaves not a protective air proof coating but a porous surface which 70 permits air to pass through it to cause further evaporation in the body of the product.

75 Among other things, I claim as my invention a product consisting of soap in solution in naphtha or other grease solvent, 80 and the process by which I produce the same, as heretofore it has been thought that soap was insoluble in such substances. The particular steps in my improved process I will hereinafter more fully describe.

85 I will now more particularly and fully describe the steps by which I produce a soap consisting of a large proportion of naphtha holding an ordinary soap base in true or colloidal solution. Although in the process hereinafter described I use naphtha, I do not limit myself to this alone as it is evident that many other grease solvents such as other petroleum derivatives, chlorin derivatives, and carbon tetrachlorid may be used equally 90 as well. It must be understood also that although by the process here described in particular the resulting soap is about of the consistency of vaseline I am not limited by it, because by changes in the kind and amount 95 of soap base and naphtha, without detracting from the spirit of my invention, the resulting product may range through all degrees of consistency and viscosity from a liquid to a solid. I heat to about 140 degrees Fahrenheit five pounds of corn oil. I heat to the same temperature a mixture of one pound eleven ounces of caustic lye (carrying 30.14% sodium oxid) and five 100 ounces water. I mix the heated corn oil with 105 the above under constant agitation and heat the resulting mixture to about 180° Fahren-

heit for about one hour or until saponification is complete. I then allow it to cool to about 160° Fahrenheit. The result is ordinary soap in a thick pasty mass and it is this 5 which I have spoken of as being the soap base of my improved product. It is evident also that other ordinary soaps may be used as soap bases for the purpose of changing the consistency of the resulting product as 10 pointed out above or for other reasons and it must be understood that I am not limited to the use of any particular one. I dissolve the soap base above described in about two pounds of alcohol. I boil the resulting thin 15 paste in a reflux condenser and add slowly, stirring constantly, about seven pounds of naphtha. The reflux condenser causes the evaporating alcohol and naphtha to condense and flow back into the liquid. The mass is 20 then allowed to cool and forms my improved soap which, having been made by the above process, has about the consistency of vaseline. In the above process the alcohol acts as a dissolving agent and by its presence as a 25 solvent for the soap base causes the alcoholic solution of soap to form a true or colloidal solution in the naphtha. Although I have specified alcohol it must be understood that I am not limited to any particular kind or 30 even to alcohol as there are many substances which have similar properties and would serve the purpose almost as well. Although in the above specification I have stated that the alcohol is introduced after 35 saponification, it is evident that without detracting from the spirit of this invention the alcohol or other substance used in its place may be introduced at some other stage in the process; for example, it may be added with 40 the lye in the process of saponification.

Although in the particular process described above, I state that about seven pounds of naphtha is added, I wish to again call attention to the fact that the amount of 45 naphtha added may be considerably larger. In fact, naphtha may be added to such an extent that ninety per cent. or ninety-five per cent. by weight of the complete product will be naphtha. When naphtha in larger 50 amounts is used, it may be necessary to increase the amount of alcohol, but I have found by experiment that the alcohol used need never be more than about eleven or twelve per cent. by weight of the final product.

My improved soap also has remarkable lathering properties, and it may be said of it that the lather is self rising, that is, that merely upon the addition of water and the 60 application of slight heat, an abundant lather

forms. This action may be more particularly explained as follows: In the manufacture of my soap, I use a relatively high test grade of naphtha or other grease solvent, that is, one which is rather volatile and will vaporize at a temperature slightly above normal. Upon the addition of water, which is a better solvent for the alcoholic solution of soap than naphtha is, such alcoholic solution of soap goes out of solution from the naphtha and into the water. Since alcohol is soluble in water in almost any quantity, and since as pointed out above, the amount of alcohol in my whole product is a relatively small quantity, the result, upon the 75 addition of water, is practically an ordinary solution of soap in water with a small amount of alcohol also dissolved in the water, and the naphtha liberated. The resulting free volatile naphtha, being free 80 from the binding influence of the alcoholic solution of soap and in the presence of heat vaporizes and forms bubbles throughout the soapy water. This is the action which is known as lathering. It is evident that the 85 liberated naphtha will not all vaporize immediately, and that some will not vaporize at all, and it is this liquid naphtha which dissolves the grease or oil on the material being cleaned and aids the soap in removing it. 90

I claim as my invention—

1. A non-liquid composition consisting of soap, alcohol and a grease solvent, such grease solvent being substantially insoluble in water, the weight of the alcohol being less and the weight of the grease solvent being more than 20% of the weight of the whole composition. 95

2. A non-liquid composition consisting of an alcoholic soap mass carrying homogeneously combined therewith a grease solvent which is substantially insoluble in water, the weight of the alcohol being less than 20% of the weight of the whole composition, whereby upon the addition of water considerable portions of the grease solvent are set free. 100

3. A non-liquid composition consisting of an alcoholic soap mass carrying homogeneously combined therewith a hydro-carbon grease solvent, the weight of the alcohol being less and the weight of the grease solvent being more than 20% of the weight of the whole composition, whereby upon the addition of water, considerable portions of the grease solvent are set free.

In witness whereof, I have hereunto subscribed my name this 15 day of January, 1916.

JOHN W. BODMAN.